

## UNITED STATES PATENT OFFICE

2,433,033

## STABILIZATION OF MOTOR FUELS

Paul L. De Verter, Baytown, Tex., assignor to  
Standard Oil Development Company, a corpora-  
tion of Delaware

No Drawing. Application November 13, 1942,  
Serial No. 465,459

5 Claims. (Cl. 44—69)

1

This invention relates to motor fuel compositions stabilized against deterioration during storage, and more particularly to such stabilization of motor fuels which contain lead alkyl anti-knock agents.

While standing in storage, some gasoline components are slowly oxidized to objectionable materials known as gums, which cause engine troubles. To determine the stability of gasolines against gum formation, there have been devised laboratory tests which are correlated to the effects of storage. These tests have been recognized to have the ability of satisfactorily evaluating storage stability for a period of two to three years, or longer, and accordingly, have been incorporated into exacting military as well as non-military specifications.

In substance, the Army-Navy "accelerated gum test" requires that a sample of gasoline having a piece of steel immersed in it be contacted with oxygen under 100 lbs./sq. in. pressure at 212° F. for 5 hours without causing the formation of more than a tolerated gum content. In order to pass strict specifications, the gum content (corrected or uncorrected, depending on the presence of tetraethyl lead) must not exceed 6 mgs./100 ml. of the fuel. These conditions are the equivalent of from about 18 months to two years of storage.

The requirements of the "accelerated gum test" are rather severe, and although they are frequently met by unleaded straight run naphthas, there are very few gasolines important in aviation fuels which can pass these tests when containing tetraethyl lead. Only some of the very purest synthetic gasoline hydrocarbons are satisfactorily stable both with and without the addition of the tetraethyl lead anti-knock agent. Due to the increased demand for leaded aviation fuels, it has become necessary to employ stabilizing inhibitors in the fuels which otherwise could not meet stability specifications. At present there are known to be several effective organic inhibitors which have gained approval for use in leaded aviation fuels, but there have been considerable efforts to determine other factors of stabilization and find other inhibitors which function to prevent oxidation of leaded aviation fuels during storage or in the "accelerated gum test" of the fuel specifications.

The invention is based upon the discovery that certain inorganic compounds represented particularly by halides of metals in groups II to IV of the Mendeleef Periodic Table are efficient inhibitors of the deterioration of leaded gasolines. A preferred metal halide for this purpose is zinc

2

chloride. About 0.2 lb. of zinc chloride in 1000 gallons of gasoline is sufficient to accomplish the desired stabilization. However, the minimum requirement for some stocks may be greater or less than this amount. The minimum amount of the metal halide inhibitor required for any fuel to pass the "accelerated gum test" can be determined by a few simple tests, and this minimum amount, which is generally at least 0.1 lb. per 1000 gallons of fuel, is sufficient to stabilize the leaded gasoline for a considerable period of time while in storage, that is, for a period of about two years of dark storage. By increasing the amount somewhat above the minimum, the extent of stabilization is also increased up to a certain degree, but it is preferred to use as small an amount of the inhibitor as is necessary, and accordingly, in using zinc chloride and similarly effective metal halide inhibitors, concentrations of about 0.2 to 0.6 lb. per 1000 gallons of fuel were found satisfactory. In such small concentrations, these inhibitors have no detrimental effect on the quality of the gasoline, such as might be detected by inspection tests for anti-knock value, copper dish gum, copper dish corrosion, the reaction test, and acidity of residue after distillation. The exact amount of stabilizer to be used may also be varied slightly according to the amount of lead alkyl anti-knock agent used, as will be discussed later.

30 Although zinc chloride has been indicated as the preferred metal halide to be used as inhibitor or stabilizer according to this invention, other metal halides may be used such as stannous chloride,  $\text{SnCl}_2$ , stannic chloride,  $\text{SnCl}_4$ , magnesium chloride,  $\text{MgCl}_2$ , and aluminum chloride,  $\text{AlCl}_3$ . Soldering fluxes comprising metal chlorides or organo-metallic chlorides alone or with hydrochloric acid may be employed as inhibiting agents. For satisfactory stabilization of gasolines with the 35 aforesaid inhibiting agents, the soluble halide content of the gasoline, when expressed as dry  $\text{HCl}$ , should be in the order of 0.05 to 0.5 pound per 1000 gallons. Although chlorine has been thus far indicated as the halogen to be present in the halide, other halogens may also be used such as bromine, iodine, and fluorine. Broadly, the halide to be used as inhibitor might be expressed by the general formula  $\text{MX}$ , where M represents a metal selected from groups II to IV of the 40 periodic table, preferably a metal in the right-hand column of those groups, and X represents one or more halogen atoms according to the valency of M. Mixtures of these various halides may also be used.

45 The inhibitor in the preferred small concen-

trations may be readily incorporated into a hydrocarbon gasoline. In adding the inhibitor in any concentration, and particularly higher concentrations, it is preferred to use a solubilizing agent which is readily miscible with the hydrocarbons and which has no detrimental effect on the quality of the fuel, e. g., low boiling alcohols, e. g., ethyl alcohol, isopropyl alcohol, etc., ketones, e. g., acetone, methyl ethyl ketone, methyl isobutyl ketone, and anti-knock ethers, e. g., di-isopropyl ether, isopropyl tertiary butyl ether, or the like. For example, zinc chloride may be dissolved in ethyl alcohol in a concentration of 4 lbs./gallon, then  $\frac{1}{20}$  of a gallon of this solution may be added to each thousand gallons of gasoline to give it a zinc chloride content of 0.2 lb./1000 gallons. As an extra precaution, a trace of hydrochloric acid or hydrogen chloride may be placed in the alcoholic solution of the metal halide to prevent any precipitation from occurring. Of course, if desired, a smaller concentration of the metal halide in alcohol may be used, such as 1 lb. or  $\frac{1}{2}$  lb. of  $\frac{1}{12}$  lb. of the stabilizer per gallon of alcohol.

From extensive experience, it has been found that a slight precipitate, white, yellow, or brown, is formed, or the gasoline sample is slightly cloudy after oxidation when the total lead and gum precipitated exceeds 6 mg./100 ml. On analysis, these precipitates show the presence of lead oxides, indicating a breakdown of the tetraethyl lead. In some of the gasoline hydrocarbons this breakdown occurs more readily than in others. In alkylates, cracked gasolines, solvent extract gasolines, and some hydrogenated polymer gasolines, the oxidation tendency is quite pronounced, and the invention is particularly applicable for use in stabilizing such fuels, although broadly it is intended to be applied to any leaded motor fuel which tends to discolor and develop a pre-

taining other lead alkyl anti-knock agents, such as lead tetramethyl or some of the intermediate or mixed methyl ethyl compounds, such as lead trimethyl monoethyl, lead dimethyl diethyl, lead monomethyl triethyl, or even lead alkyls containing higher alkyl groups than ethyl. The invention may also be applied to motor fuels containing mixtures of two or more different lead alkyl anti-knock agents. The amount of the lead alkyl agent used in the motor fuel may vary according to the anti-knock properties, generally expressed as octane number, desired in the finished fuel blend, but normally will range from about 0.5 to 3 cc. of lead alkyl per gallon of fuel, although considerably more may be used since Government specifications now permit 4 cc. per gallon at least for said military purposes. If only 1 cc. of T. E. L. (tetraethyl lead) is used per gallon of fuel, 0.1 lb. of zinc chloride per 1,000 gals. of fuel will normally suffice for stabilization, and on the other hand, with larger than normal amounts of T. E. L., e. g., 4 cc. per gallon of fuel, 0.2 to 0.4 lb. of zinc chloride per 1,000 gals. of fuel will usually be required.

The efficacy of the inorganic inhibitors was determined through the recognized accelerated gum tests and through actual storage tests. As a result of these tests, it was concluded that the inorganic inhibitors make feasible a practicable stabilization of the fuels commensurate with the effectiveness of well-known organic inhibitors.

In Table 1 is listed "accelerated gum test" data obtained on several different samples of aviation fuels containing 3.0 cc. of T. E. L. (tetraethyl lead) per gallon with varied concentrations of zinc chloride as the inhibitor. In blending the zinc chloride with the hydrocarbon fuel, a small amount of ethyl alcohol was used to dissolve the zinc chloride, and it was found that the ethyl alcohol by itself had no inhibiting effect.

Table 1

| Test No. | Type of Product<br>(contains 3.0 T. E. L. cc./gal.) | ZnCl <sub>2</sub> <sup>1</sup> Added<br>Lbs./1000 gal. | Accelerated Gum Test |                 |      |      |
|----------|-----------------------------------------------------|--------------------------------------------------------|----------------------|-----------------|------|------|
|          |                                                     |                                                        | Precipitate          | Lead and<br>Gum | Lead | Gum  |
| 1.       | 100 Octane Aviation Fuel A-1                        | 0                                                      | Hvy. Brown           | 27.9            | 15.1 | 12.8 |
| 2.       | do                                                  | 3.0                                                    | None                 | 7.3             | 4.0  | 3.3  |
| 3.       | 100 Octane Aviation Fuel A-2                        | 0                                                      | Hvy. Brown           | 43.9            | 27.2 | 16.7 |
| 4.       | do                                                  | 3.0                                                    | None                 | 7.5             | 4.0  | 3.5  |
| 5.       | Pecos Aviation Fuel B-1                             | 0                                                      | Hvy. Brown           | 36.6            | —    | —    |
| 6.       | do                                                  | 0.2                                                    | None                 | 4.3             | —    | —    |
| 7.       | do                                                  | 0.4                                                    | do                   | 3.3             | —    | —    |
| 8.       | do                                                  | 1.0                                                    | do                   | 4.5             | —    | —    |
| 9.       | Alkylate Fuel C-1                                   | 0                                                      | Hvy. Brown           | 25.8            | —    | —    |
| 10.      | do                                                  | 0.3                                                    | None                 | 6.0             | —    | —    |
| 11.      | Alkylate Fuel C-2                                   | 0                                                      | Hvy. Brown           | 31.4            | 22.8 | 8.6  |
| 12.      | do                                                  | —                                                      | do                   | 27.9            | 15.4 | 12.5 |
| 13.      | do                                                  | 0.2                                                    | None                 | 4.2             | 0.2  | 4.0  |
| 14.      | Alkylate Fuel C-3                                   | 0                                                      | Hvy. Brown           | 47.8            | 23.2 | 24.6 |
| 15.      | do                                                  | 0.05                                                   | do                   | 40.9            | 22.2 | 18.7 |
| 16.      | do                                                  | 0.10                                                   | Slt. Brown           | 11.1            | 6.4  | 4.7  |

<sup>1</sup> ZnCl<sub>2</sub> dissolved in alcohol-concentration 1 lb. ZnCl<sub>2</sub> per 12.0 gals. alcohol.

<sup>2</sup> No ZnCl<sub>2</sub> used—2.4 gal. alcohol used, the equivalent of what would be added through the use of 0.2 lb. of ZnCl<sub>2</sub> reagent.

Hvy. means heavy.

Slt. means slight.

cipitate during storage, regardless of the source of crude petroleum from which the fuel base stock was obtained, i. e., whether paraffinic, naphthenic, Mid-Continent or a synthetic fuel base stock. Light and heat act to accelerate oxidation and decomposition of tetraethyl lead in the fuel.

Although the invention has been described as applied to motor fuels containing lead tetraethyl, it is believed to apply also to fuels con-

70  
75  
The above tests show that various amounts ranging from 0.1 to 3.0 lbs. of zinc chloride per 1000 gallons of fuel were effective or entirely prevented formation of any precipitate and it substantially reduced the gum and lead deposits during the accelerated gum test. Test No. 12 shows that the amount of alcohol, used as solubilizer for the zinc chloride, does not per se have any substantial effect in reducing either the formation of a heavy brown precipitate or in

reducing the amount of lead and gum deposits in the accelerated gum test, so that it is clear that the addition of zinc chloride is responsible for the surprisingly good results obtained in the tests in which zinc chloride was used.

Another series of tests, the results of which are shown in Table 2 herebelow, were made to ascertain whether the addition of zinc chloride would have any detrimental effect on the quality of the fuel as indicated by octane number, copper dish gum, copper dish corrosion, reaction test, and acidity of residue after distillation.

Table 2

| Test No. | Sample                           | ZnCl <sub>2</sub> , Lbs./1000 g. | Octane No. | Cu Dish Gum | Cu Dish Corrosion | Reaction Test | Acidity of Residue |
|----------|----------------------------------|----------------------------------|------------|-------------|-------------------|---------------|--------------------|
| 17       | 100 Oct. Base (unleaded)         | 0                                | 86.1       | 1.2         | O. K.             | Negative      | None.              |
| 18       | do                               | 0.2                              | 86.1       | 1.6         | O. K.             | do            | Do.                |
| 19       | 100 Oct. Base + 3.0 cc. T. E. L. | 0                                | 100        | 1.7         | O. K.             | do            | Do.                |
| 20       | do                               | 0.2                              | 100        | 1.3         | O. K.             | do            | Do.                |

These tests show that the use of 0.2 lb. of zinc chloride per 1000 gallons of fuel (which as shown in Table 1 was sufficient to prevent the deterioration during storage as indicated by the accelerated gum test) had no deleterious effect on the octane number or on any of the other characteristics determined in this series of tests.

Another series of tests was made to compare the effect of zinc chloride in various concentrations on two other fuel base stocks to which 3 cc. of T. E. L. per gallon had been added, and to determine the effectiveness of various inorganic halides other than zinc chloride. The results of these tests are shown in the accompanying Table 3.

Table 3

| Test No. | Sample                             | Lbs. Inhibitor per 1000 Gallons                 | Accelerated Gum Test |              |      |      |
|----------|------------------------------------|-------------------------------------------------|----------------------|--------------|------|------|
|          |                                    |                                                 | Precipitate          | Lead and Gum | Lead | Gum  |
| 21       |                                    | 0                                               | Hy. Brown            | 37.0         | 26.8 | 10.2 |
| 22       |                                    | 0.2 ZnCl <sub>2</sub>                           | Sl. Brown            | 13.8         | 7.2  | 6.6  |
| 23       | Pecos Aviation Fuel B <sub>2</sub> | 0.4 ZnCl <sub>2</sub>                           | None                 | 6.7          | 3.7  | 3.0  |
| 24       |                                    | 1.0 ZnCl <sub>2</sub>                           | do                   | 6.2          | 3.4  | 2.8  |
| 25       |                                    | 0.5 Gal. HCl <sup>1</sup>                       | do                   | 6.9          | 4.1  | 2.8  |
| 26       |                                    | 0                                               | Hy. Brown            | 30.6         | 25.0 | 5.6  |
| 27       |                                    | 0.5 Gal. HCl <sup>1</sup>                       | None (Sl. Turbid)    | 19.2         |      |      |
| 28       |                                    | 1.0 Gal. HCl <sup>1</sup>                       | None                 | 4.2          |      |      |
| 29       |                                    | 0.4 ZnCl <sub>2</sub>                           | Hy. Brown            | 24.0         | 16.8 | 7.2  |
| 30       |                                    | 0.6 ZnCl <sub>2</sub>                           | None                 | 1.9          |      |      |
| 31       |                                    | 1.0 ZnCl <sub>2</sub>                           | do                   | 2.8          |      |      |
| 32       | Alkylate C <sub>4</sub>            | 0.6 SnCl <sub>4</sub>                           | do                   | 7.9          | Nil  | 7.6  |
| 33       |                                    | 1.0 SnCl <sub>4</sub>                           | None (Sl. Turbid)    | 4.0          | Nil  | 4.0  |
| 34       |                                    | 0.6 SnCl <sub>4</sub>                           | None                 | 7.2          | Nil  | 7.2  |
| 35       |                                    | 1.0 SnCl <sub>4</sub>                           | Trace White          | 1.7          | Nil  | 1.7  |
| 36       |                                    | 0.6 MgCl <sub>2</sub>                           | do                   | 2.0          | Nil  | 2.0  |
| 37       |                                    | 1.0 AlCl <sub>3</sub>                           | None (Sl. Rust)      | 1.5          | Nil  | 1.5  |
| 38       |                                    | 1 Gal. Soldering Flux (In alcohol) <sup>2</sup> | None                 | 4.2          |      |      |

<sup>1</sup> Gallons of 38% aqueous hydrochloric acid agitated with 1000 gallons of gasoline; most (estimated as being at least 90%) of this acid settled out and was removed from the gasoline before testing.  
<sup>2</sup> One gallon of commercial (Dewalco 52 Degree Liquid) soldering flux, comprising HCl and ZnCl<sub>2</sub>, agitated with 1000 gallons of gasoline; most of this flux (estimated as being at least 95%) settled out and was removed from the gasoline before testing.

The above tests in Table 3 indicate that with Pecos aviation fuel B<sub>2</sub> slightly more than 0.2 lb. of zinc chloride were required per 1000 gallons of fuel to prevent any brown precipitation during the accelerated storage test and to reduce the lead and gum deposits to the desired minimum during the accelerated gum test. Test No. 25 shows that washing the Pecos fuel with concentrated hydrochloric acid alone in the proportion of 0.5 gallon of acid per 1000 gallons of oil was substantially as effective as 0.4 lb. of zinc chloride per 1000 gallons of fuel. On the other hand with alkylate fuel

6 C<sub>4</sub>, as shown in tests 26-28, washing the fuel with concentrated hydrochloric acid in the proportion of 1.0 gallon of acid per 1000 gallons of oil was required to obtain satisfactory stabilization. With this same alkylate fuel, 0.6 lb. of zinc chloride per 1000 gallons of fuel was required for stabilization. Similarly, as shown in tests 32-37, 0.6 to 1.0 lb. of stannous chloride, stannic chloride, magnesium chloride, and aluminum chloride likewise produced satisfactory stabilization. According to test No. 38, washing an alkylate fuel with a commercial liquid soldering flux which contained a sub-

stantial proportion of zinc chloride and some hydrochloric acids using one gallon of flux per 1000 gallons of fuel was substantially as effective as a similar amount of straight hydrochloric acid. On the other hand, although not shown in the test, washing an alkylate fuel with a similar amount of concentrated sulfuric acid, i. e., one gallon of acid per 1000 gallons of fuel, did not prevent the formation of a precipitate and did not prevent the formation of a substantial lead deposit in the accelerated gum test. The metal chlorides are preferred to hydrochloric acid from the point of view of causing less corrosion of metals, and of all of the halides used in this series of tests the zinc chloride is the most practical.

Some preliminary storage tests were also made 65 in which 100 octane gasoline containing 3 cc. of T. E. L. was stored in brown glass bottles for thirty days with and without small iron strips which apparently acted as oxidation catalysts in increasing the severity of the deterioration. The following Table 4 shows the results of these tests before and after thirty days' storage, tests 39-41 being without any inhibitor and tests 42-44 being made with 0.4 lb. of zinc chloride per 1000 gallons of fuel under test conditions comparable 70 to those used in tests 39-41.

Table 4

| Test No. | Sample            | Inhibitor,<br>Lbs./1000<br>Gals. | Container                | Days'<br>Storage | Accelerated Gum        |            |      |      |
|----------|-------------------|----------------------------------|--------------------------|------------------|------------------------|------------|------|------|
|          |                   |                                  |                          |                  | Precipitate            | Pb+<br>Gum | Pb   | Gum  |
| 39       |                   |                                  | Brown Bottle             |                  | Heavy Brown            | 26.3       | 14.2 |      |
| 40       | 100 Oct. Gasoline | 0                                | do                       | 30               | do                     | 30.5       | 18.8 | 12.1 |
| 41       |                   |                                  | Brown Bottle + Fe Strips | 30               | do                     | 74.2       | 57.2 | 11.7 |
| 42       |                   |                                  | Brown Bottle             | 0                | None                   | 3.0        |      |      |
| 43       | 100 Oct. Gasoline | .4 ZnCl <sub>2</sub>             | do                       | 30               | do                     | 3.1        |      |      |
| 44       |                   |                                  | Brown Bottle + Fe Strips | 30               | None (Slightly Turbid) | 3.3        |      |      |

The results shown in the above Table 4 indicate that 0.4 lb. of zinc chloride per 1000 gallons of 100 octane gasoline (containing 3 cc. of tetraethyl lead per gallon) was sufficient to prevent brown precipitate formation and to prevent lead and gum deposits during the accelerated gum test, not only when tested immediately before storage but also when tested after thirty days' storage, either in the glass bottle without iron strips or in the bottle with iron strips. This is quite remarkable since the presence of the iron strips, as shown in test 41, very greatly increased the amount of lead and gum deposits in the accelerated gum test. In all three instances the use of the zinc chloride reduced the lead and gum deposits from between 26-74 down to between 3.0 and 3.3.

Although no comparable test results are available on a gasoline containing tetraethyl lead, two tests were made to determine the octane number after two years' storage of an unleaded fuel base stock with and without zinc chloride. These tests showed that without the zinc chloride the fuel had an octane number of 83.0, whereas with 0.2 lb. of zinc chloride per gallon of fuel, the octane number was 84.0, thus indicating that the zinc chloride had a partial stabilizing effect on the gasoline base stock even in the absence of tetraethyl lead. The octane number of this gasoline base stock before the two years' storage was probably about 86. Undoubtedly in view of the remarkable effectiveness of the zinc chloride as shown in Tables 1-4 in preventing a formation of a heavy brown precipitate and in reducing the lead and gum deposits in the accelerated gum tests, the octane number after two years' storage of an uninhibited fuel containing tetraethyl lead would be very much lower than the octane number of a similar fuel containing zinc chloride.

It is not intended that this invention be limited to the specific examples which have been given merely for the sake of illustration nor necessarily by any theory as to the mechanism of the operation of the invention, which is not clearly understood, but only by the appended claims in which it is intended to claim all novelty.

inherent in the invention as well as all modifications coming within the scope and spirit of the invention.

I claim:

1. A motor fuel comprising a major proportion of gasoline, about 0.5 to 6.0 cc. of tetraethyl lead per gallon of gasoline, and about 0.1 to 1.0 lb. of zinc chloride per 1000 gallons of fuel.
2. Fuel according to claim 1 also containing a small amount of organic compound selected from the group consisting of low boiling alcohols, ethers and ketones as solubilizer for the zinc chloride in the gasoline.
3. A motor fuel comprising a major proportion of aviation gasoline base stock, about 1 to 4 cc. of tetraethyl lead per gallon of gasoline, about 0.2 to 0.6 lb. of zinc chloride per 1000 gallons of fuel and a small amount of alcohol to solubilize the zinc chloride in the gasoline.
4. A motor fuel comprising a major proportion of a gasoline base stock having an octane number at least as high as 80, a sufficient amount of tetraethyl lead to raise the octane number of said gasoline base stock up to 100, and about 0.2 to 0.6 lbs. of zinc chloride per 1000 gallons of fuel.
5. A motor fuel comprising a major proportion of gasoline base stock derived by alkylation of lower olefins, about 1 to 4 cc. of tetraethyl lead per gallon of gasoline base stock and about 0.2 to 0.6 lb. of zinc chloride per 1000 gallons of fuel.

PAUL L. DE VERTER.

#### REFERENCES CITED

The following references are of record in the file of this patent:

#### UNITED STATES PATENTS

| Number    | Name    | Date          |
|-----------|---------|---------------|
| 2,067,331 | Michel  | Jan. 12, 1937 |
| 2,115,781 | Morrell | May 3, 1938   |

#### FOREIGN PATENTS

| Number  | Country       | Date         |
|---------|---------------|--------------|
| 459,270 | Great Britain | Jan. 5, 1937 |